

## UNITED STATES PATENT OFFICE

MILTON O. SCHUR AND BENJAMIN G. HOOS, OF BERLIN, NEW HAMPSHIRE, ASSIGNEES  
TO BROWN COMPANY, OF BERLIN, NEW HAMPSHIRE, A CORPORATION OF MAINE

## ART OF PREPARING NITROCELLULOSES AND RAW MATERIAL THEREFOR

No Drawing.

Application filed January 31, 1929. Serial No. 336,633.

This invention relates to the art of nitrating cellulose fiber to produce a product intended for use in the manufacture of films, lacquers, artificial silk, and the like, its object being to make possible a high yield of good quality product having a low acid retention.

In application Serial No. 140,674, filed October 9, 1926, by George A. Richter, Milton O. Schur, and Royal H. Rasch, and issued October 1, 1929, as Patent No. 1,729,628, various methods of conditioning cellulose fiber to render it more suitable as a raw material for nitration are disclosed. All those methods involve a treatment which renders the fiber less absorptive and reactive, as it has been found that the nitrating reaction is thereby modified in such a way as to result in a high yield of product having a low acid retention. The theory advanced in that case is that the sulphuric acid in the nitrating bath tends to gelatinize and to hydrolyze the cellulose fibers, especially if the pulp is highly absorptive. If, however, as explained in that application, the fiber is beaten, treated with regenerated cellulose or with nitrocellulose, or is otherwise rendered less reactive, side reactions are apparently retarded or avoided and nitration proceeds smoothly. A thin coating or film of dry nitrocellulose on the fibers, for example, probably allows nitric acid to penetrate into the fiber wall more easily than it does the sulphuric acid and perhaps readily allows water generated within the fiber during nitration to diffuse into the main body of the nitrating acid, so that within the fiber wall there is believed to be a nitric-acid-rich mixture which has a greatly reduced gelatinizing tendency and which nitrates the cellulose before hydrolysis proceeds to any troublesome degree. It is well known, for example, that nitrating acids rich in nitric acid give high yields, but that acids rich in sulphuric acid cause hydrolysis and correspondingly low yields. The thin coating or film applied to the fibers prior to nitration, by slowing up the reaction, eliminates local over-heating in the acid bath, and may also thus prevent loss in yield, for the higher the temperature of nitration, the

greater is the tendency for the yield to drop because of side reactions. Another function of the protective coating or film may be to cement the loosely adhering surface fibers to the body of the sheet or shreds of pulp, thereby counteracting the tendency of the nitrated surface fibers to pass into colloidal solution in the nitrating acid and to become lost during the separation of the spent acid from the nitrocellulose in the centrifuge.

In accordance with the process of the present invention, we treat fiber with acid-repellent material such as waxes and oils, as we have discovered that the use of a very small amount of such material results in marked improvements upon subsequent nitration of the fiber. Apparently, such materials, even when they produce an exceedingly thin coating or film on the fibers, sufficiently protect the cellulose from gelatinization and hydrolysis during nitration to bring about the desired results. Preferably, the acid-repellent material employed is free from objectionable color-yielding or stability-lowering matter,—paraffin oil, paraffin wax, and stearic acid being examples of material of this type. We believe that waxy or resinous material such as naturally occurs in the fiber exerts a protective influence during nitration, but its presence in more than traces is objectionable, because it tends to make the fiber float on the nitrating acid, with the attendant risk of pot fires and non-uniform nitration, because such material is usually associated with color-yielding compounds, and because its composition is variable and uncertain. The process of the present invention may therefore be applied to especial advantage in the case of wood pulp, particularly those pulps which have been refined to high alpha cellulose content by the removal of beta and gamma celluloses, lignin, and resins. Such purified wood pulp, by reason of its lower cost, may be used to advantage as a substitute for highly refined cotton fiber in the preparation of nitrocelluloses, but it has been found that it may under some conditions give a slightly lower yield of product than the cotton fiber. By the process of the present invention, however, the nitrating qualities of the wood fiber

may be improved at low expense to render it a more perfect raw material for nitration.

The acid-repellent material may be applied to the fiber in various ways, using liquid carrying agents, as by dispersing such material in water or dissolving in organic solvents. The carrying agent may then be removed from the fiber before nitration, as by drying, so as to avoid dilution of the nitrating acids. For instance, paraffin oil, wax, stearic acid, or like material, may be dispersed in a small amount of water containing small quantities of a soap, such as potassium oleate, as the dispersing agent. Or material such as paraffin oil or paraffin may be dissolved in a comparatively cheap volatile solvent such as gasoline. The use of dispersions in water is more economical, however, and avoids fire hazard. The fiber may be treated with the dispersion or solution of the acid-repellent material while it is in bulk, in beaten, or in unbeaten condition, or in the form of a sheet of thin paper or tissue. When treated in bulk condition, a dispersion of acid-repellent material, such as oil or wax, stabilized by soap, may be added to the pulp in the beater engine, and the oil or wax fixed on the fibers through the use of, say, alum, or other precipitating agent, in much the same way that rosin size is precipitated on pulp in the beater engine. Or, since only traces of the protective agent are needed in the fiber, the alum or other fixing agent may be omitted. The fiber may then be sheeted on a paper machine, and the paper nitrated. Or pulp may first be sheeted into paper and the sheet of paper may then be passed through a dispersion or solution of the acid-repellent material, whereupon the liquid carrier may be removed by vaporization, and the paper nitrated.

Experiment has shown that through the incorporation of as low as 0.1% paraffin wax, stearic acid, or the like, in the form of a dispersion, to comparatively free pulp, followed by the fixing of the paraffin on the fibers, the sheeting of the pulp into paper, and the nitration of the paper, we may realize yields of nitrocellulose which compare favorably with those attained when the fiber is well beaten. It is thus possible to avoid the more expensive expedient of thoroughly beating the fiber prior to sheeting into paper, in order to increase yield and at the same time produce a raw material from the comparatively free fiber as suitable as that obtained from thoroughly beaten fiber.

In order to appreciate the utility of the process of our invention, a specific example of procedure will now be given, according to which a sheet of paper made of a refined wood pulp was treated with a paraffin wax dispersion in water, dried, and then nitrated. The wood pulp employed as a raw material was a sulphite pulp which had been refined

by cooking in a caustic soda solution containing oleic acid, which served to remove beta and gamma celluloses and resinous impurities from the pulp. The pulp was then bleached and the bleached pulp sheeted into paper of 30 pounds basic weight. A dispersion of acid-repellent material was prepared by vigorously agitating a solution of paraffin wax in kerosene with a dilute solution of soap in water, whereupon the mixture was passed through a colloid mill to ensure thorough dispersion. The resulting dispersion was diluted with water until the ratio of paraffin to water was 1 to 12,000. This dilute dispersion served as a bath through which the dry sheet of paper was passed. The paper thus treated, when dried, showed no signs of wax, either in appearance or feel. When nitrated at 40° C., it gave a theoretically perfect yield of nitrocellulose which when dissolved in suitable solvents gave solutions of marked clarity and sparkle. Following are tabulated results obtained from treated and untreated papers when nitrating acid containing 20.5% HNO<sub>3</sub>, 60.8% H<sub>2</sub>SO<sub>4</sub>, and 18.7% H<sub>2</sub>O was used at 40° C. for 30 minutes:

|                                            | Untreated paper | Treated paper | 95  |
|--------------------------------------------|-----------------|---------------|-----|
| Per cent wax added to sheet                | 0               | 0.025         |     |
| Yield on nitration                         | 150.7           | 154.8         |     |
| Initial temperature rise of nitrating bath | 1.4             | 1.2           |     |
| Viscosity of nitrocellulose                | 6.7             | 8.3           |     |
| Per cent nitrogen in nitrocellulose        | 11.00           | 11.00         |     |
| Per cent theoretical yield realized        | 97.4            | 100.0         |     |
| Bursting strength of film                  | 104             | 110           |     |
| Tensile strength of film                   | 4530            | 5370          | 100 |
| Tensile stretch of film                    | 13.5%           | 20.0%         |     |

(The ratio of weight of acid to fiber was 50 to 1, and the paper was shredded into small pieces before nitration.)

It is noteworthy to remark that the shredded paper containing wax had little or no tendency to stick to the sides of the nitrating pot, whereas the run in which untreated paper was employed had to be closely watched, shreds being scraped from the sides of the pot in order to ensure complete nitration. It is noteworthy that while a slight amount of acid-repellent material such as paraffin wax effects the beneficial improvements indicated in the foregoing table, more than, say, 0.2% is apparently unnecessary and may be detrimental, in that nitration may be retarded to too great an extent and hence necessitate an excessively long time of reaction for complete nitration, and the fiber may tend to float on the acid. But with under, say, 0.1% added wax, although the reaction is slowed down materially, complete reaction is realized in a reasonable time and no serious tendency of the fiber to float is manifested. As further indicated in the table, the presence of wax in the paper improved the strength and elasticity of films prepared from the resulting nitrocellulose.

Another example of procedure according

to which dispersed paraffin wax was incorporated into pulp and fixed on the fibers before sheeting into paper and nitrating was substantially as follows. One thousand 5 pounds of refined wood pulp of the type hereinbefore described was placed in a beater engine and water disseminated therethrough to produce a stock density of about 5% (bone-dry basis). To the stock was then added 125 10 gallons of a dispersion of paraffin wax prepared by dissolving 4 1/4 pounds of wax in 9 1/2 pounds of warm kerosene, shaking vigorously with 50 pounds of warm water containing 1.9 pounds of potassium oleate dissolved therein, 15 and diluting the resulting dispersion to 125 gallons. The beater charge was brought to a slowness corresponding to slightly less than that of stock intended for bond paper, and was run directly over the paper machine. 20 The paper was found to contain about 0.1% of added wax. Upon nitrating such paper as previously described, a yield of 156.7% and a nitrogen content of 11.20 were obtained,— corresponding to a theoretical yield of 99.9%.

25 Having thus described certain embodiments of this invention, it should be evident to those skilled in the art that various changes and modifications might be made therein without departing from the spirit or scope 30 of invention as defined by the appended claims.

We claim:

1. A process which comprises treating cellulose fiber with non-cellulosic, acid-repellent material and then nitrating the fiber.
2. A process which comprises treating cellulose fiber with paraffin wax and then nitrating the fiber.
3. A process which comprises treating cellulose fiber with non-cellulosic, acid-repellent material and a liquid carrier for said material, and then nitrating the fiber.
4. A process which comprises treating cellulose fiber with non-cellulosic, acid-repellent material and a liquid carrier for said material, removing the carrier, and then nitrating the fiber.
5. A process which comprises treating cellulose fiber with an aqueous dispersion of acid-repellent material, and then nitrating the fiber.
6. A process which comprises treating cellulose fiber with an aqueous dispersion of acid-repellent material, drying, and then nitrating the fiber.
7. A process which comprises treating cellulose fiber with an aqueous dispersion of paraffin wax, drying, and then nitrating the fiber.
8. A process which comprises treating cellulose pulp with an aqueous dispersion of acid-repellent material, sheeting into paper, and nitrating the paper.
9. A process which comprises treating cellulose pulp with an aqueous dispersion of

acid-repellent material, fixing such material on the fibers, sheeting into paper, and nitrating the paper.

10. A process which comprises treating cellulose pulp with an aqueous dispersion of paraffin wax containing soap as a dispersing agent, sheeting into paper, and nitrating the paper. 70

11. A process which comprises treating cellulose pulp with an aqueous dispersion of paraffin wax containing soap as a dispersing agent, precipitating the wax on the fibers, sheeting into paper, and nitrating the paper. 75

12. A process which comprises treating paper with non-cellulosic, acid-repellent material, and then nitrating the paper. 80

13. A process which comprises treating paper with paraffin wax, and then nitrating the paper.

14. A process which comprises treating paper with a liquid carrying non-cellulosic, acid-repellent material, removing the liquid from the paper, and nitrating the paper. 85

15. A process which comprises treating paper with an aqueous dispersion of acid-repellent material, and nitrating the paper. 90

16. A process which comprises treating paper with an aqueous dispersion of acid-repellent material, drying, and nitrating the paper. 95

17. A process which comprises treating paper with an aqueous dispersion of paraffin, drying, and nitrating the paper.

18. Cellulose fiber containing less than about 0.1% by weight of acid-repellent material deposited therein. 100

19. A waterleaf paper containing less than 0.1% by weight of acid-repellent material deposited on the fibers thereof.

20. A waterleaf paper containing less than 0.1% by weight of paraffin deposited on the fibers thereof. 105

In testimony whereof we have affixed our signatures.

MILTON O. SCHUR. 110  
BENJAMIN G. HOOS.

110

115

120

125

130